

# UNITED STATES PATENT OFFICE.

STEPHEN C. BABCOCK, OF HAMBURG, AND ELMER W. HAGMAIER, OF LACKAWANNA,  
NEW YORK.

## PROCESS FOR ELECTRODEPOSITION OF COPPER.

1,174,466.

Specification of Letters Patent.

Patented Mar. 7, 1916.

No Drawing.

Application filed July 12, 1915. Serial No. 39,384.

*To all whom it may concern:*

Be it known that we, STEPHEN C. BABCOCK and ELMER W. HAGMAIER, citizens of the United States, residing at Hamburg and 5 Lackawanna, respectively, in the county of Erie and State of New York, have invented new and useful Improvements in Processes for Electrodeposition of Copper, of which the following is a specification.

10 Our invention relates to improvements in electro-deposition of copper. It is applicable generally to electro-deposition or copper plating, and is especially advantageous in making half-tones, electrotypes, in covering 15 wires for electrical conductors and for lining tanks and pipes with copper.

The object of our invention is to cut down the time necessary to get a required deposit of copper and at the same time secure a de- 20 posit that is dense and that will fill every crack and crevice, and consequently give a most perfect coating or a most perfect plate.

In carrying out our process we employ the common and well-known apparatus, which 25 needs no description.

The special and novel feature of our invention is the electro-deposition of copper from a solution containing copper sulfate, sulfuric acid, creosote, phenol, crysyl hydrate or cresylol, phlorol, and gaiacol. The 30 addition of these phenolic homologues causes a harder and firmer deposition, causes the copper to deposit in the smallest indentations, and also increases the rate of deposition. These conditions we understand 35 are brought about by the phenol homologues keeping the metal ions at a constant concentration at the cathode, and preventing all ions which usually migrate to the anode 40 from transporting electricity. It also would appear, from the perfectness of the deposition, that the addition of said ingredient prevents pocketing of gases on the cathode and thus secures a more perfect filling of all 45 interstices.

The following is a specific adaptation of

our generic invention. The bath is made up in the usual way, having about two hundred and seventy pounds of copper sulfate dissolved in about two hundred and forty gallons of water. To this is added about forty-nine ounces of phenol sulfonic acid, properly prepared so that the phenol is thoroughly combined with the sulfuric acid. The current employed is between three and 55 four volts and the amperage is about seven hundred and fifty to a two hundred and forty gallon tank. The current density is somewhat variable, and can be varied depending upon the acidity of the solution. 60

Operation and test of these improvements show a time-reduction over previously-known methods of about fifty per cent., and as above stated, the deposition is much more perfect and of greater density. 65

Having thus described our invention and its method of operation, and without limiting ourselves to the proportions, or amounts, or to any species of the genus employed, we claim:—

1. The herein described process of electro-deposition comprising adding to a copper sulfate bath a phenol compound, and applying current in the usual manner.

2. The herein described process of electro-deposition comprising adding to an ordinary sulfate of copper bath, phenol sulfonic acid in substantially the proportions above described, and applying current as described. 75

3. The herein described process of electrical deposition of copper comprising adding to an ordinary sulfate of copper bath a phenol treated with sulfuric acid in approximately the proportions above described, and applying current in the usual manner. 80

STEPHEN C. BABCOCK.  
ELMER W. HAGMAIER.

Witnesses:

ARTHUR J. MONRO,  
ARTHUR R. JENKINS.